

# United States Patent Office

3,060,098  
Patented Oct. 23, 1962

1

3,060,098

## DENTIFRICE

Sol D. Gershon, West Englewood, N.J., assignor to Lever Brothers Company, New York, N.Y., a corporation of Maine

No Drawing. Filed Nov. 18, 1957, Ser. No. 696,953  
8 Claims. (Cl. 167—93)

This invention relates to a dentifrice capable of giving a high luster to teeth and more particularly to a dentifrice having high luster-producing characteristics comprising  $\alpha$ -alumina in admixture with a polishing agent having a Mohs hardness below about 6.

Probably the most important single ingredient of a dentifrice is the polishing agent. This ingredient is in large measure responsible for the scouring and polishing action of the dentifrice. Scouring is essential to remove the more closely adherent matter and to produce a good tooth luster. In order to obtain an optimum luster effect, however, it is necessary to balance carefully the abrasive and polishing characteristics of the polishing agent. An ingredient which is quite hard will be excessively abrasive, may tend to produce grooving of the teeth, and will remove excessive amounts of enamel. On the other hand, a polishing ingredient which is too soft does not have an adequate scouring and polishing power, and will not give good tooth luster because of this deficiency. All commonly used polishing agents cause microscopic pits and scratches in the enamel, to varying degrees.

Many ingredients have been proposed as scouring and polishing agents, including calcium carbonate, the various calcium phosphates and particularly dicalcium and tricalcium orthophosphates, pumice, silica, kaolin, magnesium oxide and hydroxide, and various aluminas and alumina hydrates. The harder ingredients such as pumice tend to scratch the teeth. Aluminas in general are too abrasive and produce undue grooving and scratching. Other ingredients such as magnesium oxide may have adequate scouring power but have a disagreeable taste. It has been proposed heretofore to use microcrystalline aluminum hydroxide in major amount mixed with other somewhat harder materials, but this is relatively soft, too soft to give the desired scouring and polishing effect. None of these is entirely satisfactory from the standpoint of tooth luster.

The standardized luster test to evaluate ability to improve tooth luster in accordance with the invention is carried out as follows:

The labial surface of an extracted human central incisor is smoothed with sandpaper, ending with fine grade sandpaper, followed by levigated alumina, and then dulled by buffing with a slurry of chalk. The enamel surface then contains pits characteristic of a chalk-dulled surface. The degree of dullness is carried to a uniform low reflectance level as measured by a standardized light source-photocell assembly. The tooth is then brushed with the test composition on a standardized brushing machine for a period of two hours, following which the luster is again measured. The luster increase represents the difference between the prebrushing luster figure and the figure obtained after brushing with the test dentifrice, and is the average of the luster increase obtained on three different teeth. The measurement of luster of any one tooth is accurate within one unit. The same three teeth are used in any comparative test series.

The test dentifrice is evaluated for its tendency to pit and scratch and groove by brushing with the test dentifrice three human central incisors whose surfaces have been made absolutely pit- and scratch-free by polishing with silica.

The dentifrice composition of the instant invention comprises an  $\alpha$ -alumina having an average particle size with-

2

in the range from about 0.05 to about 5 microns, preferably from 0.2 to 1.5 microns, and a Mohs hardness of about 9, in an amount within the range from about 0.1 to about 40%, preferably 0.5 to 5%, of the total polishing agent, in combination with from 99.9 to 60%, preferably 99.5 to 95%, of one or more additional polishing agents having a Mohs hardness below about 6. Dicalcium orthophosphate dihydrate is preferred. The  $\alpha$ -alumina polishing agent of the invention is characterized by smoothly surfaced particles having rounded edges, i.e., free from sharp corners.

The polishing agent mixture in accordance with the invention gives a balanced scouring and polishing action when the  $\alpha$ -alumina and the supplemental polishing agent are present in proportions within the ranges stated. In fact, mixtures having these proportions give an optimum enamel surface substantially free from grooves, scratches and pits. The  $\alpha$ -alumina alone is very abrasive and produces very heavy enamel grooving. Dicalcium phosphate is a substance of relatively low abrasive properties, but it nonetheless can give heavy scratching and light pitting of the enamel. The mixture of both in accordance with the invention also produces an optimum luster increase or superior to that obtainable with  $\alpha$ -alumina alone.

There are many crystalline forms of alumina and it is important to distinguish these.  $\alpha$ -Alumina is anhydrous, of the formula  $Al_2O_3$ , and has a melting point of 2050° C. It is distinguished by its X-ray diffraction pattern from other aluminas, including  $\beta$ -alumina and  $\gamma$ -alumina, and from their hydrates. "Bayer process alumina" is the  $\alpha$ -trihydrate (page 5, Technical Paper No. 10, entitled "Alumina Properties," by Allen A. Russell, published by the Aluminum Company of America, and Industrial and Engineering Chemistry 37, 796-802 (1945)). The "Bayer process alumina" described in the Atkins Patent No. 2,010,910 is a calcined  $\alpha$ -trihydrate, probably having a water content within the range  $Al_2O_3 \cdot 0.5H_2O$  to  $Al_2O_3 \cdot 3H_2O$ . Aluminum hydroxide is another name for the  $\alpha$ -trihydrate, an antecedent before calcining of  $\alpha$ - and  $\gamma$ -alumina. Calcining the  $\alpha$ -trihydrate for one hour at about 1150° C. produces  $\alpha$ -alumina, and calcining at 450° C. produces  $\gamma$ -alumina which is hygroscopic.

An especially preferred  $\alpha$ -alumina for use in accordance with the invention is Linde Type A  $\alpha$ -alumina abrasive. This material is an  $\alpha$ -alumina available commercially, having an approximate average particle size of 0.3 micron, an apparent density of 0.3 to 0.6 g. per c., and a melting point of 2050° C., and is characterized by smooth-surfaced particles having round edges. It has a hardness of 9 on Mohs' scale, corresponding to corundum. Linde Type C is the same as Type A but has an average particle size of 1 micron.

The  $\alpha$ -alumina employed in the compositions of the invention is obtainable by calcining ammonium aluminum sulfate, usually in the form of ammonium alum, its dodecahydrate, at temperatures in excess of 1150° C. but well below the fusion point of  $\alpha$ -alumina, preferably about 1175° C. Calcining at such temperatures avoids fusion of the mass and yields a powdered product of the desired particle size, namely, within a range from 0.05 to 5 microns, and the particles have rounded edges, whereas pulverization produces particles having sharp edges.

In addition to the  $\alpha$ -alumina, which is present in only a small amount, there is employed another polishing agent having a Mohs hardness below about 6. The preferred supplemental polishing agent is dicalcium orthophosphate dihydrate. There can also be used tricalcium orthophosphate and calcium pyrophosphate, as well as an insoluble sodium polymetaphosphate, calcium carbonate, magnesium oxide and magnesium carbonate. These can be used alone or in admixture; the insoluble sodium poly-

metaphosphate would usually be used with a calcium or magnesium phosphate or carbonate.

The dentifrice usually will contain from about 20% to about 99.5% total of the polishing agent, depending upon the physical state of the dentifrice. Preferably from 40 to 60% is used in a tooth paste and from 88 to 98% in a tooth powder; of this, from 0.1 to 40% will be  $\alpha$ -alumina and from 99.9 to 60% other polishing agents.

In addition to the polishing agent, the dentifrice can contain as optional ingredients a soap or synthetic detergent as a surface tension depressant, flavoring materials, oxygen-releasers, such as perborates, buffers, sweeteners, such as saccharin, harmless coloring materials, in proportions to give any desired effect. These are conventional components of dentifrices, and materials suitable for this purpose need not be enumerated, for they are well known to those skilled in the art.

In a preferred embodiment of the invention, the dentifrice is in the form of a paste, and in this event it will contain a carrier and softener and a binder in amounts to give the dentifrice a smooth texture and good flowability. Glycerin and sorbitol are preferred carriers and softeners, but ethyl alcohol, mineral oil, syrup, glucose and invert sugars, glycols and honey can also be employed. As binders there can be used gum tragacanth, sodium carboxymethylcellulose, Indian gum, Irish moss and its derivatives, starch, acacia gums, agar agar, locust bean gum, pectin and petrolatum. Those skilled in the art know other carriers and softeners, and binders.

The dentifrice also can contain therapeutic agents such as tryothrycin, chlorophyllins, hexachlorophene, the sarcosides, and water-soluble ionizable fluoride compounds, and the amount is not critical but will be enough to obtain a beneficial effect. Usually an amount within the range from about 0.01 to about 2% by weight of the dentifrice is sufficient. The fluoride content is calculated as fluoride ion. The alkali metal fluorides are conveniently available and would ordinarily be employed. Sodium fluoride, sodium fluostannite, lithium fluoride, stannous fluoride, stannous chlorofluoride, potassium fluoride and ammonium fluoride are typical of the members of this class.

The following are general formulations of tooth pastes and powders coming within the scope of the invention:

#### TOOTH PASTE

|                            | Percent by weight |                 |
|----------------------------|-------------------|-----------------|
|                            | Permissible range | Preferred range |
| Total polishing agent      | 20 to 80          | 40 to 60        |
| $\alpha$ -alumina          | 0.05 to 20        | 0.25 to 2.5     |
| Other polishing agent      | 19.05 to 60       | 39.75 to 57.5   |
| Carrier and softener       | 5 to 70           | 15 to 40        |
| Binder                     | 0.5 to 30         | 0.7 to 5        |
| Miscellaneous              | 5 to 70           | 15 to 40        |
| Flavor                     | 0.1 to 5          | 0.8 to 2        |
| Water                      | 4 to 60           | 15 to 30        |
| Surface tension depressant | 0.01 to 6         | 0.5 to 3.5      |
| Buffers                    | 0.02 to 10        | 0.1 to 2        |
| Preservative               | 0.01 to 1         | 0.1 to 0.3      |

#### TOOTH POWDER

|                            | Percent by weight |                 |
|----------------------------|-------------------|-----------------|
|                            | Permissible range | Preferred range |
| Total polishing agent      | 88 to 99.5        | 88 to 98        |
| $\alpha$ -Alumina          | 0.1 to 40         | 0.5 to 5        |
| Other polishing agent      | 82.9 to 59.5      | 87.5 to 93      |
| Miscellaneous              | 0.5 to 10         | 2 to 4          |
| Flavor                     | 0.01 to 5         | 1 to 3          |
| Surface tension depressant | 0.01 to 6         | 0.5 to 3.5      |
| Buffers                    | 0.02 to 10        | 0.1 to 2        |

The following examples represent in the opinion of the inventor preferred embodiments of his invention:

#### Examples 1 to 12

A group of dicalcium phosphate dentifrices was made up according to the following formulation:

|    | Ingredients                            | Parts by weight |                  |
|----|----------------------------------------|-----------------|------------------|
|    |                                        | Control A       | Examples 1 to 12 |
| 10 | Dicalcium phosphate dihydrate          | 47.57           | 47.07            |
|    | $\alpha$ -Alumina as stated in Table I |                 | 0.50             |
| 15 | Sodium caragheenate                    | 1.00            | 1.00             |
|    | Aqueous sorbitol solution, 70%         | 20.64           | 20.64            |
|    | Polyethylene glycol 400                | 4.26            | 4.26             |
|    | Glycerin                               | 4.33            | 4.38             |
| 20 | Distilled water                        | 19.88           | 19.88            |
|    | Sodium lauryl sulfate                  | 1.17            | 1.17             |
|    | Flavor                                 | 1.10            | 1.10             |
|    |                                        | 100.00          | 100.00           |

These dentifrices were subjected to the luster test with the following results. Surface effects evaluation was done by microscopic examination at a magnification of 57 $\times$ :

Table I

| Example No. | Abrasive                  | X-ray analysis       | Luster increase | Surface effects                                            |
|-------------|---------------------------|----------------------|-----------------|------------------------------------------------------------|
| 30          | Dicalcium phosphate.      | -----                | 33              | Heavy scratching, light pitting.                           |
| 1           | Linde Type A              | $\alpha$ -Alumina    | 53              | Light scratching, slight pitting.                          |
| 2           | Alcoa A5                  | do                   | 37              | Heavy scratching, very heavy pitting, moderate grooving.   |
| 35          | Alcoa A10                 | do                   | 38              | Heavy scratching, very heavy pitting, moderate grooving.   |
| 40          | Alcoa A14                 | do                   | 36              | Heavy scratching, heavy pitting, moderate grooving.        |
| 45          | Alcoa A302                | do                   | 36              | Very heavy scratching, moderate grooving.                  |
| 5           | Alcoa T60                 | do                   | 32              | Very heavy grooving.                                       |
| 6           | Alcoa T61                 | do                   | 31              | Very heavy scratching, heavy pitting, very heavy grooving. |
| 50          | Norton 600X               | do                   | 39              | Very heavy scratching.                                     |
| 8           | Norton 38600X             | do                   | 38              | Very heavy scratching, very heavy grooving.                |
| 9           | Norton 38900              | do                   | 37              | Very heavy scratching, very heavy pitting, heavy grooving. |
| 55          | Kaiser alumina hydrate.   | $\alpha$ -Trihydrate | 42              | Heavy pitting, heavy grooving.                             |
| 10          | Reynolds alumina hydrate. | $\beta$ -Trihydrate  | 42              | Heavy pitting, moderate grooving.                          |
| 11          |                           |                      |                 |                                                            |
| 60          |                           |                      |                 |                                                            |

The table shows the improvement in tooth luster-producing effectiveness of the dicalcium phosphate dentifrices which result from the addition of 0.5% of the alumina given in the table. The dentifrice containing the Linde Type A  $\alpha$ -alumina abrasive in accordance with the invention gave an almost glass smooth tooth surface, free from grooves and practically free of pits and scratches, and a luster increase of 53. The other dentifrices tested were markedly inferior, giving a tooth surface marked with a multitude of microscopic pits, scratches, and grooves, and a luster increase as low as 31, well below Control A.

## Examples 13 to 16

Four dicalcium phosphate tooth paste formulations were prepared using from 0.25 to 1%  $\alpha$ -alumina having the following formulation:

| Ingredients                    | Example No. |        |        |        |
|--------------------------------|-------------|--------|--------|--------|
|                                | 13          | 14     | 15     | 16     |
| Linde Type A $\alpha$ -alumina |             | 0.25   | 0.50   | 1.00   |
| Dicalcium phosphate dihydrate  | 47.57       | 47.32  | 47.07  | 46.57  |
| Sodium carrageenate            | 1.00        | 1.00   | 1.00   | 1.00   |
| Aqueous sorbitol solution, 70% | 20.64       | 20.64  | 20.64  | 20.64  |
| Polyethylene glycol 400        | 4.26        | 4.26   | 4.26   | 4.26   |
| Glycerin                       | 4.38        | 4.38   | 4.38   | 4.38   |
| Distilled water                | 19.89       | 19.89  | 19.89  | 19.89  |
| Sodium lauryl sulfate          | 1.17        | 1.17   | 1.17   | 1.17   |
| Flavor                         | 1.09        | 1.09   | 1.09   | 1.09   |
|                                | 100.00      | 100.00 | 100.00 | 100.00 |

The luster increase was as follows:

| Ex. No. | Abrasive                                                                  | Luster increase |
|---------|---------------------------------------------------------------------------|-----------------|
| 13      | Dicalcium phosphate                                                       | 33              |
| 14      | Mixture of dicalcium phosphate and Linde Type A $\alpha$ -alumina, 0.25%. | 53              |
| 15      | Mixture of dicalcium phosphate and Linde Type A $\alpha$ -alumina, 0.5%.  | 56              |
| 16      | Mixture of dicalcium phosphate and Linde Type A $\alpha$ -alumina, 1.0%.  | 57              |

It is apparent that even 0.25%  $\alpha$ -alumina (Example 14) gives a remarkable improvement as compared to the formulation with only dicalcium phosphate as the abrasive (Example 13). Doubling the amount of  $\alpha$ -alumina to 0.5% (Example 15) gives a somewhat better luster increase, and doubling it again (Example 16) gives another increment in luster increase.

It is apparent that as the amount of  $\alpha$ -alumina increases beyond 0.5%, the improvement in luster increase is not commensurate with the greater amount of  $\alpha$ -alumina required, showing that small amounts, which are more economical, would usually be adequate.

## Example 17

Two dicalcium phosphate formulations were prepared as follows:

| Ingredients                        | Percent by weight |        |
|------------------------------------|-------------------|--------|
|                                    | A                 | B      |
| Linde Type $\alpha$ -alumina       |                   | 0.10   |
| Dicalcium orthophosphate dihydrate | 49.63             | 49.53  |
| Sodium carrageenate                | 0.95              | 0.95   |
| Aqueous sorbitol solution, 70%     | 19.72             | 19.72  |
| Polyethylene glycol 400            | 4.07              | 4.07   |
| Glycerin                           | 4.38              | 4.38   |
| Distilled water                    | 19.01             | 19.01  |
| Sodium lauryl sulfate              | 1.17              | 1.17   |
| Flavor                             | 1.07              | 1.07   |
|                                    | 100.00            | 100.00 |

Formulation B gave a luster increase of 49, as compared to 37 for formulation A.

Teeth brushed with the dentifrice containing  $\alpha$ -alumina had a smoother surface than the teeth brushed with the control paste which did not contain  $\alpha$ -alumina. Moreover, the tooth surfaces brushed with the  $\alpha$ -alumina dentifrice were relatively free from microscopic scratches and pits characterizing tooth surfaces brushed with the control dentifrice.

## Example 18

The following is an example based on a mixture of di-

calcium phosphate dihydrate and dicalcium phosphate anhydrous as the supplemental polishing agents:

| 5                               | Ingredients | Percent by weight |      |
|---------------------------------|-------------|-------------------|------|
|                                 |             | A                 | B    |
| Dicalcium phosphate dihydrate   | 42.72       | 41.72             |      |
| Dicalcium phosphate, anhydrous  | 5.00        | 5.00              |      |
| $\alpha$ -Alumina, Linde Type A |             | 1.00              | 1.00 |
| Sodium carrageenate             | 20.64       | 20.64             |      |
| Aqueous sorbitol solution, 70%  | 4.26        | 4.26              |      |
| Polyethylene glycol 400         | 4.27        | 4.27              |      |
| Glycerin                        | 19.90       | 19.90             |      |
| Distilled water                 | 1.13        | 1.13              |      |
| Sodium lauryl sulfate           | 1.08        | 1.08              |      |
| Flavor                          |             |                   |      |
|                                 | 100.00      | 100.00            |      |

Formulation A produced a luster increase of 43. Substituting 1%  $\alpha$ -alumina for an equal amount of dicalcium phosphate dihydrate gave a luster increase of 57, 14 points higher.

Teeth brushed with the dentifrice containing  $\alpha$ -alumina had a smoother surface than the teeth brushed with the control paste which did not contain  $\alpha$ -alumina. Moreover, the tooth surfaces brushed with the  $\alpha$ -alumina dentifrice were relatively free from the microscopic scratches and pits characterizing tooth surfaces brushed with the control dentifrice.

## Example 19

In the following example tricalcium phosphate is used as the supplemental polishing agent:

| 35                              | Ingredients | Percent by weight |   |
|---------------------------------|-------------|-------------------|---|
|                                 |             | A                 | B |
| Tricalcium phosphate            | 36.20       | 35.20             |   |
| $\alpha$ -Alumina, Linde Type A | 1.00        | 1.00              |   |
| Gum tragacanth                  | 23.60       | 23.60             |   |
| Glycerin                        | 29.29       | 29.29             |   |
| Distilled water                 | 3.00        | 3.00              |   |
| Urea                            | 5.00        | 5.00              |   |
| Diammonium phosphate            | 0.96        | 0.96              |   |
| Sodium lauryl sulfate           | 0.95        | 0.95              |   |
| Flavor                          |             |                   |   |
|                                 | 100.00      | 100.00            |   |

Formulation A gave a luster increase of 43, whereas formulation B gave a luster increase of 54, 11 points higher.

Teeth brushed with the dentifrice containing  $\alpha$ -alumina had a smoother surface than the teeth brushed with the control powder containing no  $\alpha$ -alumina. Moreover, the tooth surfaces brushed with the  $\alpha$ -alumina dentifrice were relatively free from the microscopic scratches and pits characterizing tooth surfaces brushed with the control dentifrice.

## Example 20

A calcium carbonate type formula was made up as follows:

| 60                                       | Ingredients | Percent by weight |   |
|------------------------------------------|-------------|-------------------|---|
|                                          |             | A                 | B |
| Calcium carbonate (chalk, light, U.S.P.) | 46.98       | 46.48             |   |
| $\alpha$ -Alumina, Linde Type A          | 31.39       | 31.39             |   |
| Glycerin                                 | 18.40       | 18.40             |   |
| Distilled water                          | 1.01        | 1.01              |   |
| Sodium lauryl sulfate                    | 1.20        | 1.20              |   |
| Sodium carrageenate                      | 1.02        | 1.02              |   |
| Flavor                                   |             |                   |   |
|                                          | 100.00      | 100.00            |   |

Formula A gave a luster increase of 26, and formulation B a luster increase of 51, an increase of 25 points.

Teeth brushed with the dentifrice containing  $\alpha$ -alumina had a smoother surface than the teeth brushed with the

control powder containing no  $\alpha$ -alumina. Moreover, the tooth surfaces brushed with the  $\alpha$ -alumina dentifrice were relatively free from the microscopic scratches and pits characterizing tooth surfaces brushed with the control dentifrice.

*Example 21*

A calcium pyrophosphate tooth paste was prepared as follows:

| Ingredients                     | Percent by weight |        |
|---------------------------------|-------------------|--------|
|                                 | A                 | B      |
| Calcium pyrophosphate           | 45.27             | 44.77  |
| $\alpha$ -Alumina, Linde Type A | 0.50              |        |
| Sodium carrageenate             | 1.30              | 1.30   |
| Glycerin                        | 23.18             | 23.18  |
| Distilled water                 | 27.98             | 27.98  |
| Sodium lauryl sulfate           | 1.17              | 1.17   |
| Flavor                          | 1.10              | 1.10   |
|                                 | 100.00            | 100.00 |

Formulation A had a luster increase of 40, and formulation B a luster increase of 52, 12 points higher.

Teeth brushed with the dentifrice containing  $\alpha$ -alumina had a smoother surface than the teeth brushed with the control paste which did not contain  $\alpha$ -alumina. Microscopic scratches and pits were reduced in number, compared with the control dentifrice.

*Example 22*

A dicalcium phosphate dihydrate tooth powder having the following formulation was prepared:

| Ingredients                     | Percent by weight |        |
|---------------------------------|-------------------|--------|
|                                 | A                 | B      |
| Dicalcium phosphate dihydrate   | 96.85             | 95.85  |
| $\alpha$ -Alumina, Linde Type A | 1.00              |        |
| Sodium lauryl sulfate           | 1.25              | 1.25   |
| Flavor                          | 1.90              | 1.90   |
|                                 | 100.00            | 100.00 |

Formulation A gave a luster increase of 39, whereas formulation B was 16 points higher, or 55.

Teeth brushed with the dentifrice containing  $\alpha$ -alumina had a smoother surface than the teeth brushed with the control powder containing no  $\alpha$ -alumina. Moreover, the tooth surfaces were relatively free from the microscopic scratches and pits characterizing tooth surfaces brushed with the control dentifrice.

*Example 23*

Four different tooth paste formulations were made up, two containing a mixture of dicalcium phosphate and Linde Type A  $\alpha$ -alumina abrasive, another identical with this but without the  $\alpha$ -alumina abrasive, and a third which did not contain any dicalcium phosphate, but in which the  $\alpha$ -alumina abrasive constituted the sole polishing agent. These dentifrices had the following formulation:

| Ingredients                        | Parts by weight |        |        |        |
|------------------------------------|-----------------|--------|--------|--------|
|                                    | A               | B      | C      | D      |
| Linde Type A $\alpha$ -alumina     | 39.77           | 0.50   | 10.00  |        |
| Dicalcium orthophosphate dihydrate | 49.63           | 49.13  | 37.20  |        |
| Sodium carrageenate                | 0.95            | 0.80   | 0.95   | 0.90   |
| Aqueous sorbitol solution, 70%     | 19.72           | 24.31  | 19.72  | 20.87  |
| Polyethylene glycol 400            | 4.07            | 5.03   | 4.07   | 4.31   |
| Glycerin                           | 4.38            | 4.38   | 4.38   | 4.38   |
| Distilled water                    | 19.01           | 23.43  | 19.01  | 20.09  |
| Sodium lauryl sulfate              | 1.17            | 1.17   | 1.17   | 1.17   |
| Flavor                             | 1.07            | 1.11   | 1.07   | 1.08   |
|                                    | 100.00          | 100.00 | 100.00 | 100.00 |

These paste dentifrices were tested for luster increase, abrasion (enamel loss) and surface effects. Abrasion

testing was done by measuring the thickness of extracted human teeth before and after each brushing with a given dentifrice; any differences represented enamel loss. The test was as developed by G. H. Wandel. The test tooth was first conditioned by storage in tap water until the thickness measurements were constant and remained constant for three successive days. The tooth was mounted in the bottom of a metal cup directly below a revolving brush of the type used by dentists in prophylactic work.

The slurry of the test product was then poured into the cup and the machine was operated. The cup and tooth were moved slowly back and forth beneath the revolving brush for a period of one hour. The tooth thickness was then remeasured. The abrasion loss represents the difference between the initial and final measurement of tooth thickness. Results on three teeth were averaged to obtain the abrasion loss value. This test is reported in chapter 15, "Dentifrices," by S. D. Gershon, H. H. Pokras, and T. H. Rider, of the text *Cosmetics: Science and Technology*, by Sagarin, Interscience Publishers (1957). Surface effects evaluation was done by microscopic examination at a magnification of 57 $\times$  of teeth brushed with dentifrices containing each of the abrasives indicated.

TABLE II

|                                                                          | Abrasive | Luster increase | Abrasion (enamel loss), mm.                             | Surface Effects |
|--------------------------------------------------------------------------|----------|-----------------|---------------------------------------------------------|-----------------|
| 30                                                                       |          |                 |                                                         |                 |
| (A) Dicalcium phosphate                                                  | 37       | Nil             | Heavy scratching, light pitting.                        |                 |
| (B) Linde Type A $\alpha$ -alumina                                       | 52       | .073            | Slight scratching, slight pitting, very heavy grooving. |                 |
| 35 (C) Mixture of dicalcium phosphate and Linde Type A $\alpha$ -alumina | 53       | .001            | Minimum of scratching, minimum of pitting.              |                 |
| (D) Mixture of dicalcium phosphate and Linde Type A $\alpha$ -alumina    | 54       | .0033           | Slight scratching, light grooving.                      |                 |
| 40                                                                       |          |                 |                                                         |                 |

The above results show that a tooth paste composed wholly of dicalcium phosphate is a nonabrasive, low luster producer which causes heavy scratching and light pitting (dentifrice A). An abrasive composed entirely of the Linde Type A  $\alpha$ -alumina is a good luster producer but it is very abrasive and causes very heavy enamel grooving (dentifrice B). Dentifrices composed of a mixture of dicalcium phosphate and 0.5% and 10% Linde Type A  $\alpha$ -alumina abrasives are relatively nonabrasive, excellent luster producers which leave a minimum of enamel surface markings with only light scratching and slight pitting (dentifrices C and D). The Luster Increase is much higher than would be expected for the amount of  $\alpha$ -alumina that is present (only 0.5% in dentifrice C) and the enamel loss also is less than would be expected, particularly in dentifrice C, and the surface is better as well, being smooth and virtually pit-, groove- and scratch-free.

Increasing the amount of  $\alpha$ -alumina in D to 10%, i.e., twenty times C, gave only a small Luster Increase as compared to C, and a considerably greater enamel loss with light grooving. This shows the desirability of employing a minimum amount of the  $\alpha$ -alumina, since the smaller amounts give practically as good a Luster Increase without undesirable side effects. This confirms the preference for an amount within the range from 0.5 to 5%  $\alpha$ -alumina by weight of the total polishing agent. However, obviously considerably more  $\alpha$ -alumina could have been used without obtaining undue abrasion and heavy grooving.

It will be evident to those skilled in the art that many variations can be made in the compositions of the dentifrice of the invention and accordingly the invention is

not to be limited except as set forth in the appended claims.

All parts and percentages in the specification and claims are by weight.

I claim.

1. A dentifrice capable of imparting an improved luster increase to teeth with a minimum of surface enamel markings including pits, scratches and grooves, said dentifrice being composed of from about 20% to about 99.5% by weight of a polishing agent consisting essentially of from about 0.1% to about 40% by weight of anhydrous alpha-alumina composed of smoothly surfaced particles having rounded edges of an average particle size within the range of from about 0.05 to about 5 microns, a density of about 0.3 to 0.6 gram per cubic centimeter, and a Mohs hardness of about 9, and from about 99.9% to about 60% by weight of a supplemental polishing agent having a Mohs hardness below about 6 and selected from the group consisting of dicalcium phosphate, tricalcium phosphate, calcium pyrophosphate and calcium carbonate.

2. A dentifrice in accordance with claim 1 in which the supplemental polishing agent is dicalcium phosphate.

3. A dentifrice in accordance with claim 1 in which the supplemental polishing agent is tricalcium phosphate.

4. A dentifrice in accordance with claim 1 in which the supplemental polishing agent is calcium pyrophosphate.

5. A dentifrice in accordance with claim 1 in which the supplemental polishing agent is calcium carbonate.

6. A paste dentifrice in accordance with claim 1 including from about 20% to about 85% by weight of the polishing agent, from 5% to 70% by weight of a carrier and from 0.5% to 30% by weight of a binder.

7. A powder dentifrice in accordance with claim 1

35 pp. 13, 15 and 17.

comprising from 83% to 99.5% by weight of the polishing agent.

8. A dentifrice capable of imparting an improved luster increase to teeth with a minimum of surface enamel markings including pits, scratches and grooves, said dentifrice being composed of from about 20% to about 99.5% by weight of a polishing agent consisting essentially of from about 0.25% to about 5% by weight of anhydrous alpha-alumina composed of smoothly surfaced particles having rounded edges of an average particle size within the range of from about 0.2 micron to about 1.5 microns, a density of about 0.3 to 0.6 gram per cubic centimeter, and a Mohs hardness of about 9, and from about 99.5% to about 95% by weight of a supplemental polishing agent having a Mohs hardness below about 6 and selected from the group consisting of dicalcium phosphate, tricalcium phosphate, calcium pyrophosphate and calcium carbonate.

#### References Cited in the file of this patent

#### UNITED STATES PATENTS

|           |                |       |               |
|-----------|----------------|-------|---------------|
| 2,010,910 | Atkins         | ----- | Aug. 13, 1935 |
| 2,359,326 | Moss et al.    | ----- | Oct. 3, 1944  |
| 2,550,207 | Tainter et al. | ----- | Apr. 24, 1951 |

#### OTHER REFERENCES

Frary: Ind. Eng. Chem., vol. 38 (1946), pp. 129-132.  
Stumpf et al.: Ind. Eng. Chem., vol. 42, July 1950, pp. 1398-1403.

30 Ray: Dental Cosmos, November 1933, pp. 1070-1077.  
Bailey: Journal of Dental Research, December 1950, pp. 740-748.

Russell: Technical Paper No. 10, Alumina Properties, Aluminum Co. of America, Pittsburgh, Pa., April 1953,